

## UNITED STATES PATENT OFFICE.

NINO MAGELSEN, OF CHRISTIANIA, NORWAY.

## PROCESS OF PRODUCING A FIREPROOF AND ELASTIC MATERIAL.

1,074,511.

Specification of Letters Patent. Patented Sept. 30, 1913.

No Drawing.

Application filed November 23, 1911. Serial No. 661,934.

*To all whom it may concern:*

Be it known that I, NINO MAGELSEN, a subject of the King of Norway, residing at Christiania, Norway, have invented certain new and useful Improvements in the Process of Producing a Fireproof and Elastic Material; and I do hereby declare the following to be a full, clear, and exact description of the invention, such as will enable others skilled in the art to which it appertains to make and use the same.

This invention relates to compositions of materials and has for its object a process of producing a fireproof material, which is elastic and able to resist the action of water and acids, and which may be employed for providing various objects made for instance of wood, metals, burnt clay, cement, plaster of Paris, with a protective covering.

20 The main components from which the material is produced are carbonate of lime, water-glass and asbestos.

The process of producing the material is preferably carried out in the following manner. Carbonate of lime in the form of chalk, together with a suitable amount of asbestos, is mixed with water-glass to form a uniform mixture to which a small amount of an acid or substances acting as an acid upon

30 the water glass are added and incorporated in the mass. The amounts of the various components are so proportioned as to obtain a mass of pasty consistence. It is of importance, that the water-glass (double

35 water-glass) employed, contains an excess of alkali or some alkali should be mixed

with it. It has been found, in most cases, that an excess of alkali of about 13 per cent. (preferably 8 per cent. KOH and 5 per cent.

40 NaOH) will be sufficient. The acid (or acid substance) introduced into the composition acts to initiate the reaction which is completed later on, when the composition is subjected to the action of the carbon di-

45 oxid of the atmosphere. As an acid substance may be advantageously employed, I use a ferrous sulfate containing acid in excess, and of this substance 3.5 per cent. may be employed.

50 When this composition is to be used for

providing objects of various materials with a protective covering the pasty mass is spread upon the object in a layer of suitable thickness, whereupon the object is placed so as to be subject to the action of the air. In certain cases it will be suitable to maintain the coating heated for some time. The composition will then after a short time be transformed into a hard covering, which is at the same time elastic, and which will adhere to the underlayer with great strength. The covering obtained in this manner is fireproof and resists the action of warm as well as of cold water and of cold or boiling dilute and concentrated acids.

The relative amounts of the various components of the composition is to be varied in accordance to the special use in each case and to the method employed in spreading the composition upon the object to be coated, as this may be effected in various manners for instance by means of a brush or the like.

As the covering is in itself hard and elastic the objects which are provided with this covering may be very thin and it is also possible to produce objects of various shapes from a composition as that above described without the use of other materials.

The covering may advantageously be employed upon vessels (for instance cooking vessels) of metals or burnt clay instead of the enamel or lead glass usually employed for this purpose.

80 I claim:  
The process of producing a fireproof and elastic material capable of resisting the action of water, which consists in mixing carbonate of lime and asbestos with waterglass containing an excess of alkali, and incorporating in the mass a substance acting as an acid upon the silicate.

90 In testimony that I claim the foregoing as my invention, I have signed my name in presence of two subscribing witnesses.

NINO MAGELSEN.

Witnesses:

MARTIN E. GUTTORMSEN,  
HENRY BONLEWICH.